# EUROPEAN PATENT SPECIFICATION

(11) **EP 2 862 645 B1**
(45) Date of publication and mention of the grant of the patent: **22.01.2020**
(21) Application number: 13179299.6
(22) Date of filing: 05.08.2013
(51) Int. Cl.: B21B 1/16, E04C 5/01, B21F 9/00, B21C 43/04

(54) **METHOD, APPARATUS AND ARRANGEMENT FOR MANUFACTURING REINFORCEMENT STEEL, AND REINFORCEMENT STEEL MANUFACTURED THEREWITH**
VERFAHREN, VORRICHTUNG UND ANORDNUNG ZUR HERSTELLUNG VON BETONEISEN UND DAMIT HERGESTELLTE BETONEISEN
PROCÉDÉ, APPAREIL ET SYSTÈME DE FABRICATION D'ACIER D'ARMATURE ET LEDIT ACIER

(30) Priority: 03.08.2012 NL 2009282
(43) Date of publication of application: 22.04.2015
(73) Proprietor: Znd Draad B.V., 5555 XD Valkenswaard (NL)
(72) Inventor: van Beek, Wilhelmus Josephus, 5555XD Valkenswaard (NL)
(74) Representative: V.O.

(56) References cited:
- EP-A1- 0 601 630
- EP-A1- 0 806 257
- WO-A1-99/41029
- WO-A2-00/06317
- GB-A- 2 214 846
- US-A- 4 216 666
- Anonymous: "BS 4449", , 23 May 2008 (2008-05-23), XP055488488, Retrieved from the Internet: URL:https://www.concretecentre.com/Concret e-Design/Design-Codes/BS-4449.aspx [retrieved on 2018-06-27]

## Description

### Field of the invention

The present invention is directed to a method of manufacturing reinforcement steel for reinforcement of concrete structures, said reinforcement steel having an elongated shape of arbitrary length and cross-section, said method comprising the steps of: providing a steel base wire; and rolling the steel base wire for modifying a cross-sectional dimension thereof, and for creating a bonding profile on a surface of said wire.

The invention is further directed to a manufacturing arrangement for performing the method described.

### Background

Roughly since the second half of the twentieth century, concrete has become the preferred choice of building material for building all kinds of structures. Its popularity is evidently based on the fact that it is conveniently mouldable in any preferred shape (enabling for example prefabrication) while at the same time it provides a very strong and durable building material.

An important factor in providing the strength and robustness of concrete is the use of embedded reinforcement steel inside the concrete. The reinforcement steel for example determines how well a concrete structure can withstand vibrations or shocks. To this end, the industry and governmental bodies have defined standards for the use of various kinds of reinforcement steel for different purposes. For example, an office building in an arbitrary environment and subject to average weather and geologic conditions (i.e. a low risk area) may safely be build using concrete with reinforcement steel having relatively relaxed properties with respect to its yield strength. On the other hand, a highway bridge to be built for spanning a ravine in an area where earthquakes are known to happen from time to time, must be designed to withstand the most extreme conditions. Such a bridge may be built using concrete with reinforcement steel with excellent properties with respect to tensile strength and yield strength.

Since the production method of reinforcement steel plays an important role in determining the properties of the end product, until recently, the European standards for reinforcement steel distinguished the reinforcement steel types based on their manner of manufacturing. As known to the skilled person, if reinforcement steel is manufactured and rolled at high temperatures in a blast-furnace, the properties with respect to the capacity to withstand vibrations and tensile forces improve. Therefore, the former classification well distinguished the high-grade reinforcement steel types from the lower-grade types. However, this manner of standardizing also comes with disadvantages. For example, although one would expect that the furnace based production methods usually provide high-grade metals, the classification leaves room for errors - i.e. furnace manufactured reinforcement steel being of accidental low-grade due to errors in the production process. Moreover, this standardisation only enabled the definition of two classes, being FeB500HKN (low grade) and FeB500HK/HWL (high grade) where the indications HKN, HK and HWL indicated the production process.

Since recently, the standardization has been adapted and is now only based on the properties of the end product. The existing European norms presently categorizes reinforcement steel types in three different ductility classes, being B500A, B500B and B500C, where the classes A and B more or less correspond to the earlier two classes and the additional class B500C is a new class indicating very high grade reinforcement steel. Where the number 500 in fact indicates the mandatory yield strength of the reinforcement steel (which must be 500 MPa or higher), the classes further define the property ranges in terms of two parameters: the tensile strength to yield strength ratio Rₘ/Rₑ, and the percentage uniform elongation at maximum force Agt. These latter two parameters are different for each of the classes B500A, B500B and B500C.

Existing methods for production of reinforcement steel are not really different from how it has been done for years; only the standardization has changed. This comes to no surprise, since the technical reality has not changed either. It is still furnace based manufacturing methods that enable to provide reinforcement steel types that satisfy the requirements of high grade steel types in classes B500B and C. The cold methods performed at room temperatures on steel base wire give rise to micro fractures, making the steel more prone to metal fatigue. An example of such a micro fracture can be seen in figure 6 (inside the white circle), which provides a photo taken with a scanning electron microscope of a micro fracture at the surface of a reinforcement steel wire. In this respect, it is to be noticed that the cold methods differ from the furnace based methods in that the rolling step for imprinting a profile on the wire is performed outside a furnace. In the furnace based methods, the rolling step is performed inside a furnace and an axial stretching step is performed after leaving the furnace.

A disadvantage of the present manufacturing methods for making high grade reinforcement steel of class B500B, however, is that furnace based processing steps leave a thin oxidation layer on the surface of the reinforcement steel. By performing the rolling process inside the furnace, causes the reinforcement steel to have an irregular cross-sectional shape. This is known to be problematic when the reinforcement steel is later processed after manufacturing (e.g. when being lashed or otherwise handled by a client). On the other hand, the existing cold processes only yield low grade reinforcement steel types, and cannot be applied for achieving the more stringent requirements in terms of material properties required for B500B type steel.

Documents EP0806257, EP0601630, GB2214846, WO99/41029, US4216666, and WO00/06317, relate to metal processing.

### Summary of the invention

In view of the above, it is an object of the present invention to provide a method of manufacturing high grade reinforcement steel that may be performed at low temperatures, preferably room temperature. It is a further object of the invention to provide such a method enabling at least the production of reinforcement steel satisfying the standard for B500B type steels.

The above mentioned objects of the invention are achieved in that there is provided a method of manufacturing reinforcement steel for reinforcement of concrete structures, the method being according to claim 1, said reinforcement steel having an elongated shape of arbitrary length and cross-section, said method comprising the steps of: providing a steel base wire; and rolling the steel base wire for modifying a cross-sectional dimension thereof, and for creating a bonding profile on a surface of said wire, wherein said step of rolling is a cold rolling step; characterized in that, prior to the step of rolling, the method further comprises a step of: surface layer breaking for breaking of a surface layer, and surface cleaning of said steel base wire for removing the surface layer from said steel base wire; and wherein, subsequent to said step of rolling, the method further comprises a step of applying a plurality of bending actions to the steel base wire for improving tensile properties thereof, such as to provide said reinforcement steel having a tensile strength to yield strength ratio Rₘ/Rₑ of at least 1,08, and having a percentage uniform elongation at maximum force A_{gt} of at least 5,0.

The threshold properties for providing B500B type standardized reinforcement steel is that the parameter tensile strength to yield strength ratio Rₘ/Rₑ of the reinforcement steel is at least 1,08 as presently defined, and that the percentage of total or uniform elongation at a maximum force A_{gt} is at least 5,0. For reinforcement steel on a roll the latter, the uniform elongation at a maximum force A_{gt}, must even be 5,5. As will be appreciated although these thresholds are not expected to be redefined in the future, these thresholds are merely definitions following from agreement between industry and governmental bodies which may be subject to change.

The inventive concept surprisingly has found a manner of fabricating high grade reinforcement steel satisfying the requirements for at least class B500B, wherein the step of rolling of the reinforcement steel may be performed at low temperatures (i.e. outside (or after the steel base wire has left) the furnace). The inventive manner as described above is based on insight in the material processes taking place in a steel wire upon bending the wire. The inventors have recognised that after applying just a few bending actions the properties of the metal wire in terms of the above mentioned parameters will in fact improve. This can surprisingly be applied successfully to such an extend that it becomes possible to create reinforcement steel falling within the class requirements for B500B. This process enables to improve the properties of steel base wire in such a manner that a B500B class type reinforcement steel wire may be achieved using a cold process. Whereas existing methods for manufacturing these kinds of reinforcement steel rely on a hot rolling step inside a furnace, as will be appreciated, the inventive cold process provides an important technological advantage which allows the reinforcement steel to be produced having a more accurately defined cross-sectional shape. Preferably, the bending actions are applied to the steel base wire after the step of rolling the steel base wire has been concluded.

By definition, whether a rolling process is either a cold rolling process or a hot rolling process is determined by the temperature at which the rolling process takes place in relation to the recrystallization temperature of the kind of steel to be rolled at the given ambient pressure. A cold rolling process, such as the rolling step used in the method of the present invention, takes place at a temperature below the recrystallization temperature of the steel. Any temperature below the recrystallization temperature at the given ambient pressure will be suitable, including atmospheric pressures and temperatures (these are evidently most preferred).

The advantages of the method of the present invention are evident. This is due to the fact that heating of the wire in a furnace leaves a thin and irregular layer of metal oxide on the surface of the steel wire. When rolling is performed inside the furnace, the oxidation surface layer will be present on the outer surface of the acquired shape provided by the rolling mill. This weak brittle surface layer easily comes off the surface of the wire in use, yielding a reinforcement steel wire with a slight irregular shape. By performing the rolling step outside the furnace, the oxidation layer already comes off upon cold handling of the steel base wire, and the shape is imprinted more accurately. The subsequent bending actions allow to achieve the material properties required for B500B type steel. A further advantage of the invention is that the process requires less steps and is overall more easy to perform than a furnace based process.

Conventionally, the oxidation layer is at least partly removed at some point during the process by performing a surface layer breaking step, regardless of whether the process is a cold or warm production process. In accordance with the invention, a further improvement of the production process has surprisingly be found. In accordance with a specific embodiment of the present invention, a further improvement of the method is achieved by performing an additional step of surface cleaning prior to the step of rolling, for removing a surface layer such as an oxidation layer from the steel base wire. This step of surface cleaning, although the specific type of surface cleaning may be chosen freely by the skilled person, may comprise for example a step of brushing, polishing, spooling of the wire, a chemical treatment such as staining or a high pressure fluid jet for cleaning the wire. The conventional surface breaking step removes the major part of the oxidation layer, however, it will leave remnants of the oxide layer on the surface of the steel base wire. Upon performing the cold rolling step, the rolling process pushes these small remnant parts of the oxidation layer into the steel underneath the surface, creating very small micro fractures, such as depicted in figure 6 (inside the white circle). These micro fractures have a negative effect on the strength of the reinforcement steel created.

The inventors have recognized that the properties with respect to metal fatigue of the reinforcement steel are greatly improved by complete removing the oxidation layer prior to rolling of the steel base wire, which may be achieved by performing an additional cleaning step in addition to the surface breaking step.

By removing the oxidation layer using an additional step of surface cleaning, the above mentioned effect is prevented from happening, yielding a stronger end product which is less prone to metal fatigue. As a result, the requirements of the high grade class B500B are more easily achieved using a cold process in accordance with the present invention, including the additional surface cleaning step.

As described above, the properties of the reinforcement steel rods of the present invention with respect to tensile strength to yield strength ratio and percentage uniform elongation at maximum force, are sufficiently improved for producing reinforcement steel rods of grade B500B and better using a cold rolling process in accordance with the method steps of the invention. However, although the obtained performance is good with respect to the these material properties, the cold rolling step that is applied for imprinting the profile diminishes the performance with respect to metal fatigue in comparison with conventional hot rolling processes. Imprinting the desired bonding profile on the surface of the steel wire in a cold rolling mill unit introduces sharp edges and areas of tensile stress on the surface of the wire. These sharp edges and areas of tensile stress have a negative effect on the strength of the reinforcement steel wire created. Cracks promulgate easily in areas of tensile stress because the tensile stresses are already working to pull the atoms of the metal apart. The sharp edges and corners of the imprinted profile act as potential starting points for cracks. This problem appears to be absent in hot rolling processes.

The requirements with respect to metal fatigue for reinforcement steel rods for building purposes are stringent. The table below provides the requirements with respect to metal fatigue for reinforcement steel rods having a diameter D≤28mm (table 1) and D>28mm (table 2). The term 2^{∗}σₐ relates to the amount of stress applied during the tests.
D≤28mm:

**Table 1**

| | | | |
|---|---|---|---|
| 2*σₐ = 175 MPa | | 2*σₐ = 200 MPa | |
| Number of samples: 10 ²⁾ | | Number of samples: 8 ²⁾ | |

| No. of actions *10⁶ | No. broken samples | No. of actions *10⁶ | No. broken samples |
|---|---|---|---|
| < 1,5 | None allowed | < 0,75 | None allowed |
| < 2,0 | ≤ 1 sample | 0,75 ≤ n <1,0 | ≤ 1 sample |
| ≥ 2,0 | ≥ 9 samples | 1,0 ≤ n < 2,0 | ≤ 2 samples ¹⁾ |
| | | ≥ 2,0 | ≥ 5 samples |
| 1) ≤ 3 samples in case no break occurred at up to 1,0 * 10⁶ applied action | | | |
| 2) Total number of samples: 10 + 8 = 18 | | | |

D>28mm

**Table 2**

| | | | |
|---|---|---|---|
| 2*σₐ = 145 MPa | | 2*σₐ = 170 MPa | |
| Number of samples: 10 ²⁾ | | Number of samples: 8 ²⁾ | |

| No. of actions *10⁶ | No. broken samples | No. of actions *10⁶ | No. broken samples |
|---|---|---|---|
| < 1,5 | None allowed | < 0,75 | None allowed |
| < 2,0 | ≤ 1 sample | 0,75 ≤ n <1,5 | ≤ 1 sample |
| ≥ 2,0 | ≥ 9 samples | 1,5 ≤ n < 2,0 | ≤ 2 samples ¹⁾ |
| | | ≥ 2,0 | ≥ 4 samples |
| 1) ≤ 4 samples in case no break occurred at up to 1,5 * 10⁶ applied action | | | |
| 2) Total number of samples: 10 + 8 = 18 | | | |

The method of the present invention, in accordance with a preferred embodiment, comprises a step of shot peening of the steel base wire subsequent to applying the bending actions. The inventors have recognized that the material properties with respect to metal fatigue of the cold rolled reinforcement steel rods are greatly improved by performing the step of shot peening.

Shot peening is a cold-working process in which the rolled wire is bombarded with small spherical media called shot. By shot peening the material a layer of compressive stress is introduced by compacting the material. As the shot peening is performed, the atoms on the surface of the metal become crowded, i.e. locally concentrated, and try to restore the metal's original shape, i.e. the original lattice structure, by pushing outward. The atoms deeper into the metal are pulled toward the surface by their bonds with the atoms in the compressive layer. These deeper atoms resist the outward pull creating internal tensile stress that keeps the part in equilibrium with the compressive stress on the surface. On the other hand tensile stress near the surface is relieved by the step of shot peening. Moreover the sharp edges and corners of the profile are rounded. The latter reduces the number of cracks and microfractures that may occur in these locations, while the reduced tensile stress near the surface decreases the chance that any micro fractures may propagate. As a result, the requirements of the high grade class B500B are more easily achieved using a cold process in accordance with the present invention, including the additional shot peening step.

Tests were performed on two reinforcement steel samples manufactured with process embodiments as described herein with and without a step of shot peening. Using a working stroke ('Schwingbreite', applied stress) of 260 MPa. the sample created without a step of shot peening was destroyed as a result of metal fatigue after approximately 600.000 stroke cycles. The sample created using the process including shot peening was put to the same test with the same working stroke; however this latter sample survived over 10.000.000 stroke cycles without breaking, after which the test was stopped leaving the reinforcement steel in tact.

In the method of the present invention, a number of cold-working process steps are combined in a specific sequence. By combining these steps in the sequence indicated, a high-grade type reinforcement steel wire may be obtained that is conventionally only obtainable using a hot rolling process.

In accordance with another aspect of the invention there is provided a manufacturing arrangement with the features of claim 7, for the manufacturing of reinforcement steel using a method in accordance with the first aspect, said arrangement comprising: a lead-in unit for receiving a steel base wire; and a rolling mill unit for a rolling the steel base wire for modifying a cross-sectional dimension thereof, and for creating a bonding profile on a surface of said wire; said arrangement characterized by further comprising an apparatus in accordance with the second aspect for applying a plurality of bending actions to the steel base wire for improving tensile properties thereof, such as to provide said reinforcement steel having a tensile strength to yield strength ratio Rₘ/Rₑ of at least 1,08, and having a percentage uniform elongation at maximum force A_{gt} of at least 5,0.

### Brief description of the drawings

The invention will further be elucidated by description of some specific embodiments thereof, making reference to the attached drawings, wherein:
Figure 1 schematically provides an overview of the method steps of the present invention;
Figure 2 schematically illustrates the steps of brushing and rolling of a steel base wire which may be used in accordance with the method of the present invention;
Figure 3 schematically illustrates an apparatus for applying bending actions in accordance with the present invention;
Figure 4 schematically illustrates how the rollers of the apparatus for applying and bending actions maybe adjusted relative to each other, in accordance with the present invention;
Figure 5 illustrates a manufacturing arrangement in accordance with the present invention;
Figure 6 provides a photo taken with an electron microscope of a micro fracture in the surface of a steel wire.

### Detailed description

Figure 1 illustrates a method in accordance with the present invention. The method that starts in step 2 with the providing of a steel base wire e.g. to a production line in accordance with the present invention. The steel base wire itself is usually created using a furnace based process which leaves, as an undesired side-effect, a thin irregular oxidation layer on the surface thereof. In step 3, the surface layer is broken, e.g. by twisting or vibrating the wire. In step 4, a further step of surface cleaning is performed in order to remove the oxidation layer from the surface of the steel base wire. Although the description below implements the step of surface cleaning by a step of brushing of the steel base wire, the skilled person will appreciate that many alternatives exist for performing a surface cleaning step, including but not limited to polishing, spooling, chemical cleaning e.g. by applying a stain or coating, or blowing using a high pressure fluid (such as air of water).

In step 6, a rolling action is performed on the steel base wire from a plurality of sides, for modifying the shape of the cross section or a dimension thereof (i.e. decreasing its diameter), and for imprinting a bonding profile on the surface of the wire. The bonding profile is important for providing a good bonding between the concrete and the reinforcement steel in use.

After the step of rolling of the steel base wire, the method in accordance with the present invention continues by a step 8 of applying a plurality of bending actions to the steel base wire for improving the tensile properties thereof. The bending actions are performed in the strain hardening regime of plastic deformation of the wire. As will be appreciated, this process maybe controlled in a number of ways, e.g. by increasing the number of bending actions while decreasing the intensity of the bending actions. It has been found that applying a multiple of five bending actions provides good results with the method of the present invention. However, this should not be considered as a limitation to the invention and desired results may be achieved upon applying a total of three, four, six, seven, eight, or any other number of bending actions.

After applying the bending actions in step 8, the method of the present invention continues by applying a shot peening process step 9. The shot peening step 9 improves the properties of the reinforcement steel amongst others with respect to metal fatigue, by bombarding the surface with spherical media. This relieves tensile stress near the surface and rounds the corners and edges of the profile, making the reinforcement steel less prone to metal fatigue. The method then continues by winding the reinforcement steel on a spindle in step 10, after which a manufacturing method is completed (12).

The steps 4 and 6 are schematically illustrated in figure 2. A steel base wire 15 moved in the direction of arrow 16 through a cleaning unit 17 and through a rolling mill unit 30. The surface cleaning unit 17 exists, in the present embodiment, of three steel brushes 18, 19 and 20. On the circumferential surfaces of the steel brushes 18, 19 and 20 a plurality of brush hairs generally indicated by reference numeral 23 on brush 18 extend radially there from. The brush hairs 23 strike upon rotation of the brushes 18, 19 and 20 in the direction indicated for example by arrows 25 and 26 on the surface of the steel base wire 15, removing the oxidation layer. Good results have been achieved by rotating the brushes 18, 19 and 20 in counter direction to the direction of movement of the steel wire 15. This is indicated by the arrows 25 and 26. As will be appreciated, the brushes 18, 19, and 20 may also rotate in the other direction, and the number of brushes may differ from what is indicated in figure 2. Instead of or in addition to steel brushes, a plurality of polishing brushes may be applied.

In rolling mill unit 30 a plurality of rollers 33, 34 and 35 circumferentially apply a rolling action to the surface of the steel base wire 15. Each of the rollers 33,34 and 35 comprises a slightly rounded inward shape such as is indicated for roller 35 in the dashed circle 40 by reference numeral 42. In addition, the circumferential sides of each of the rollers 33, 34 and 35 is comprised of a plurality of surface structures 43 which create the desired bonding profile on the surface of the steel wire 15 by imprinting the pattern on the surface thereof. Arrows 37 and 38 indicate the direction of rotation of roller wheels 33 and 35. Roller wheel 34 rotates in a corresponding direction as roller wheels 33 and 35.

Figure 3 schematically illustrates an apparatus for applying a plurality of bending actions in accordance with the present invention. This apparatus maybe used for applying step 8 in the method illustrated schematically in figure 1. The apparatus consists of a frame 46 which is fixedly connected to the ground 48 such as to prevent moving thereof in use. Extending from the base structure 46 an additional top structure 50 is present for supporting a second suspension unit 52 in an adjustable manner as will be explained below.

The bending actions itself are applied by a plurality of roller wheels 57, 58, 59, 60 and 61. The roller wheels are rotatable in a single plane of rotation, and are alternately suspending from shafts at either a first or a second height. The shafts extend transverse to the plane of rotation from a respective first or second suspension 53, 52. The roller wheels 57, 59, 60 and 61 are suspended from shafts from a first height. These shafts are in turn rotatably or operationally connected to a first suspension unit 53 attached to the frame structure 46 of the apparatus 45. The roller wheels 58 and 60 are suspended from shafts that are in turn operatively connected to a second suspension unit 52 which is adjustably suspended from the top frame structure 50 of the apparatus 45. The adjustable suspension of the second suspension unit 52 is provided by a hydraulic cylinder 55 which allows for adjusting the heights of roller wheels 58 and 60 above the level of roller wheels 57, 59 and 61 as will be explained below in connection with figure 4.

In order to apply the bending action, the sum of the radiuses of each two consecutive roller wheels 57-61 will be at least equal to or greater than the height of the shafts of wheels 58 and 60 above the level of the shafts of wheels 57, 59 and 61. In terms of the wording used in connection with figure 4, the sum of the radiuses of two consecutive wheels (e.g. r₁ and r₂ in figure 4) is greater than or equal to the pitch distance d₁. In test performed by the inventors, working with five roller wheels, good results have been achieved using wheels having a diameter of 150 mm (i.e. r=75 mm), a height d₁ ∼ 50 mm and a pitch distance d₂ = 150 mm. In addition, good results have been achieved with r = 125 mm, d₁ ∼ 50 mm, and d₂ = 250 mm, and with r = 130 mm, d₁ = 70 mm, and d₂ = 250 mm. As will be appreciated, these are mere test results, and the invention can be applied across a much wider range of values for r, d₁ and d₂.

In general, it is important that a number of bending actions is applied, while the exact number of bending actions, and the intensity of each bending action (determined by r, d₁ and d₂) will differ dependent on the type of steel and should be determined experimentally (e.g. by trial and error). The invention is not to be interpreted as limited to a particular choice of these parameters. To this end, it is also important to mention that the above dimensions have been used for the embodiment as illustrated in figure 3. However, performing bending action may be performed in a different manner than as specifically illustrated in figure 3. The skilled person will appreciate that a wire may be moved across the outer circumferences of a number of wheels having smaller dimensions, instead of the illustrated embodiment wherein the wire moves in between the consecutive wheels. Moreover, the bending actions may not even be performed all in a single plane of rotation.

In use, the steel base wire 15, after leaving the roller mill unit 30, will be guided via pulleys 64 and 65 to the roller wheels 57, 58, 59, 60 and 61. Each roller wheel 57-61 will apply a single bending action to the steel base wire 15 as indicated in figure 3. After applying the bending actions the steel base wire 15 is guided via pulleys 66 and 67 to a spindle (not shown in figure 3).

Figure 4 schematically illustrates how the rollers wheels of the apparatus for applying the bending action 45 maybe adjusted in use. As schematically illustrated in figure 4, each of the rollers 57, 59 and 61 suspends from a corresponding shaft 77, 79 and 81, and the midpoints of the shafts 77, 79 and 81 are aligned on a notional first line 70. Roller wheels 58 and 60 are suspended from shafts 78 and 80 which are in turn aligned on notional second line 72. The height between the first line 70 and the second line 72, d₁, is adjustable by means of the second suspension unit 52 and the hydraulic cylinder 55. In addition, each of the shafts 77, 78, 79, 80 and 81 is respectively connected to the first or second suspension unit 53 or 52 in such a manner that the position of the shaft along either the first line 70 or the second line 72 may be adjusted such as to adjust the distance d₂ between each to consecutive rollers. Moreover, the suspension of each of the roller wheels 57-61 from the shafts 77-81 is such that the roller wheels 57-61 are connected in a releasable manner such as to allow replacement of the roller wheels 57-61 by different roller wheels. This may be used for adapting the diameter of the wheels. As will be appreciated the manner in which apparatus 45 allows for adjustment of the various dimensions of the roller wheels 57-61 and their suspension relative to each other, allows for accurate dimensioning of the bending actions applied by the apparatus during the manufacturing method.

Figure 5 schematically illustrates a manufacturing arrangement in accordance with the present invention disclosing a first spindle 92 comprising a steel base wire which is fed to the arrangement at the input thereof. Prior to the surface cleaning step, surface layer breaking unit 93 twists or vibrates the wire such as to break and partly remove the brittle oxidation layer on the surface. Instead of vibrating or twisting, the steel base wire may already be moved across one or more roller wheels for breaking the surface layer. Unit 94 provides the additional surface cleaning by means of a step of brushing, e.g. as indicated in figure 2 schematically. The rolling of the steel base wire is performed by a roller mill unit 96, after which the steel base wire is provided to the apparatus for applying the bending action schematically illustrated by 98. After leaving apparatus 98 the reinforcement steel wire is lead to the second spindle 100 after which the manufacturing method is completed.

Figure 6 illustrates a micro fracture at the surface of a steel wire. The micro fracture can be clearly seen inside the wide dashed circle in the picture, and has been discussed herein above.

The present invention has been described in terms of some specific embodiments thereof. It will be appreciated that the embodiments shown in the drawings and described here and above are intended for illustrative purposes only, and are not by any manner or means intended to be restrictive on the invention. The context of the invention discussed here is merely restricted by the scope of the appended claims.

## Claims

1. Method of manufacturing reinforcement steel for reinforcement of concrete structures for providing said reinforcement steel having a tensile strength to yield strength ratio Rₘ/Rₑ of at least 1,08, and having a percentage uniform elongation at maximum force A_{gt} of at least 5,0, said reinforcement steel having an elongated shape of arbitrary length and cross-section, said method comprising the steps of:
providing (2) a steel base wire (15); and
rolling (6) the steel base wire (15) for modifying a cross-sectional dimension thereof, and for creating a bonding profile on a surface of said wire (15), wherein said step of rolling (6) is a cold rolling step;
**characterized in that**, prior to the step of rolling, the method further comprises a step of:
surface layer breaking (3) for breaking of a surface layer, and
surface cleaning (4) of said steel base wire (15) for removing the surface layer from said steel base wire (15); and
wherein, subsequent to said step of rolling, the method further comprises a step (8) of applying a plurality of bending actions to the steel base wire (15) for improving tensile properties thereof.

2. Method according to claim 1, further comprising a step of shot peening (9) subsequent to said step of applying the bending actions.

3. Method according to claim 1 or 2, wherein said bending actions are applied by moving the steel base wire (15) across a plurality of consecutive roller wheels (57, 58, 59, 60, 61), wherein for each roller wheel for providing the bending action the steel base wire (15) is moved across or with at least a part of a circumference of the wheel.

4. Method according to claim 3, wherein each roller wheel (57, 58, 59, 60, 61) is rotatable in a plane of rotation of the plurality of roller wheels, each roller wheel being rotatable by means of a shaft, and wherein from the plane of rotation of the roller wheels the shafts alternately extend transverse to the plane of rotation from positions along a first and a second line respectively, the first and the second line being parallel to each other and to the plane of rotation, wherein for each two consecutive roller wheels the sum of radiuses of the roller wheels is larger than or equal to a distance between the first and second line for forcing said bending action upon the steel base wire upon moving the wire across or with the circumference of the roller wheels.

5. Method according to any of the previous claims, wherein the step (8) of applying a plurality of bending actions comprises applying at least three bending actions.

6. Method according to any of the previous claims, wherein said additional step of surface cleaning comprises at least one step selected from a group comprising brushing, polishing, spooling of the steel base wire, a chemical treatment such as staining, or a high pressure fluid jet for cleaning the steel base wire.

7. Manufacturing arrangement for the manufacturing of reinforcement steel for reinforcement of concrete structures having a tensile strength to yield strength ratio Rₘ/Rₑ of at least 1,08, and having a percentage uniform elongation at maximum force A_{gt} of at least 5,0, using a method in accordance with at least one of the claims 1-6, said arrangement comprising:
a lead-in unit for receiving a steel base wire (15); and
a rolling mill unit (96) for applying a cold rolling step for rolling the steel base wire for modifying a cross-sectional dimension thereof, and for creating a bonding profile on a surface of said wire;
said arrangement **characterized by** further comprising, in use upstream of said rolling mill (96), a surface cleaning unit (94) for applying surface cleaning of said steel base wire prior to said step of rolling for removing a surface layer such as an oxidation layer from said steel base wire (15); and, in use downstream of said rolling mill, a bending unit (98) for applying a plurality of bending actions to the steel base wire for improving tensile properties thereof.

8. Manufacturing arrangement in accordance with claim 7, further comprising a surface layer breaking unit (93) upstream of said surface cleaning unit (94) for applying a step of surface layer breaking for breaking of a surface layer of the wire (15).

9. Manufacturing arrangement in accordance with claim 7 or 8, further comprising a shot peening unit downstream of said bending unit for applying a step of shot peening subsequent to said step of applying the bending actions.

10. Manufacturing arrangement in accordance with any of the claims 7-9, the bending unit (98) comprising a plurality of consecutive roller wheels (57, 58, 59, 60, 61) arranged in a single plane of rotation, wherein each roller wheel is rotatable by means of a shaft (77, 78, 79, 80, 81) such as to be rotatable in the plane of rotation of the plurality of roller wheels, said roller wheels being placed such that in use for providing the bending action the steel base wire is moved across or with at least a part of the circumference of each wheel.

11. Manufacturing arrangement in accordance with claim 10, wherein from the plane of rotation the shafts (77, 78, 79, 80, 81) of the roller wheels (57, 58, 59, 60, 61) alternately extend transverse to the plane of rotation from positions along a first (70) and a second line (72) respectively, the first (70) and the second line (72) being parallel to each other and to the plane of rotation, wherein for each two consecutive roller wheels the sum of radiuses of the roller wheels is larger than or equal to a distance between the first and second line for forcing said bending action upon the steel base wire upon moving the across or with the circumference of the roller wheels.

12. Manufacturing arrangement in accordance with claim 11, wherein the shafts (77, 79, 81) extending from the first line (70) are structurally connected by a first suspension unit, and wherein the shafts (78, 80) extending from the second line (72) are structurally connected by a second suspension unit, wherein at least one of the first and second suspension units is adjustably connected to a structure of the apparatus such as to enable adjustment of the distance between the first (70) and second line (72) in use.

13. Manufacturing arrangement in accordance claim12, wherein one or more of the shafts (77, 78, 79, 80, 81) is adjustably connected to the first or second suspension unit, for enabling adjustment of the position of the one or more shafts along the first or second line respectively.

14. Manufacturing arrangement in accordance with any of the claims 10-13, wherein the roller wheels (57, 58, 59, 60, 61) are suspended to the shafts (77, 78, 79, 80, 81) in a releasable manner such as to enable replacement thereof, for adapting a diameter of one or more rollers wheels (57, 58, 59, 60, 61) in use.

## Patentansprüche

1. Verfahren zur Herstellung von Bewehrungsstahl zur Bewehrung von Betonkonstruktionen zum Bereitstellen des Bewehrungsstahls mit einem Verhältnis der Zugfestigkeit zur Streckgrenze Rₘ/Rₑ von wenigstens 1.08 und einer prozentualen gleichmäßigen Dehnung bei einer maximalen Kraft A_{gt} von wenigstens 5,0, wobei der Bewehrungsstahl eine längliche Form von beliebiger Länge und Querschnitt aufweist, wobei das Verfahren die folgenden Schritte umfasst:
Bereitstellen (2) eines Stahlbasisdrahtes (15); und
Walzen (6) des Stahlbasisdrahtes (15) zum Modifizieren seiner Querschnittsabmessung und zum Erzeugen eines Verbindungsprofils auf einer Oberfläche des Drahtes (15), wobei der Schritt des Walzens (6) ein Kaltwalzschritt ist;
**dadurch gekennzeichnet, dass** das Verfahren vor dem Schritt des Walzens ferner einen folgenden Schritt umfasst:
Brechen einer Oberflächenschicht (3) zum Brechen einer Oberflächenschicht und
Oberflächenreinigung (4) des Stahlbasisdrahtes (15) zum Entfernen der Oberflächenschicht von dem Stahlbasisdraht (15); und
wobei das Verfahren nach dem Schritt des Walzens ferner einen Schritt (8) zum Anwenden mehrerer Biegewirkungen auf den Stahlbasisdraht (15) zum Verbessern seiner Zugeigenschaften umfasst.

2. Verfahren nach Anspruch 1, ferner umfassend einen Schritt des Kugelstrahlens (9) nach dem Schritt des Anwendens der Biegewirkungen.

3. Verfahren nach Anspruch 1 oder 2, wobei die Biegewirkungen durch Bewegen des Stahlbasisdrahtes (15) über mehrere aufeinanderfolgende Walzenräder (57, 58, 59, 60, 61) aufgebracht werden, wobei für jedes Walzenrad zum Bereitstellen der Biegewirkung der Stahlbasisdraht (15) über oder mit wenigstens einem Teil eines Umfangs des Rades bewegt wird.

4. Verfahren nach Anspruch 3, wobei jedes Walzenrad (57, 58, 59, 60, 61) in einer Rotationsebene der mehreren Walzenräder rotierbar ist, wobei jedes Walzenrad mittels einer Welle rotierbar ist und wobei sich von der Rotationsebene der Walzenräder die Wellen abwechselnd quer zur Rotationsebene von Positionen entlang einer ersten bzw. einer zweiten Linie erstrecken, wobei die erste und die zweite Linie parallel zueinander und zur Rotationsebene sind, wobei für jeweils zwei aufeinanderfolgende Walzenräder die Summe der Radien der Walzenräder größer oder gleich einem Abstand zwischen der ersten und der zweiten Linie ist, um die Biegewirkung auf den Stahlbasisdraht zu erzwingen, wenn der Draht über oder mit dem Umfang der Walzenräder bewegt wird.

5. Verfahren nach einem der vorhergehenden Ansprüche, wobei der Schritt (8) des Anwendens mehrerer Biegewirkungen das Anwenden von wenigstens drei Biegewirkungen umfasst.

6. Verfahren nach einem der vorhergehenden Ansprüche, wobei der zusätzliche Schritt der Oberflächenreinigung wenigstens einen Schritt umfasst, der aus einer Gruppe ausgewählt ist, die das Bürsten, Polieren, Spulen des Stahlbasisdrahtes, eine chemische Behandlung, wie beispielsweise Beizen, oder einen Hochdruck-Flüssigkeitsstrahl zum Reinigen des Stahlsockeldrahtes umfasst.

7. Herstellungsanordnung zur Herstellung von Bewehrungsstahl zur Bewehrung von Betonkonstruktionen mit einem Verhältnis der Zugfestigkeit zur Streckgrenze Rₘ/Rₑ von wenigstens 1,08 und einer prozentualen gleichmäßigen Dehnung bei einer maximalen Kraft A_{gt} von wenigstens 5,0, unter Verwendung eines Verfahrens nach wenigstens einem der Ansprüche 1 bis 6, wobei die Anordnung Folgendes umfasst:
eine Einführeinheit zur Aufnahme eines Stahlbasisdrahtes (15); und
eine Walzwerkseinheit (96) zum Anwenden eines Kaltwalzschritts zum Walzen des Stahlbasisdrahtes zum Modifizieren seiner
Querschnittsabmessung und zum Erzeugen eines Verbindungsprofils auf einer Oberfläche des Drahtes;
wobei die Anordnung **dadurch gekennzeichnet ist, dass** sie im Gebrauch stromaufwärts des Walzwerks (96) eine Oberflächenreinigungseinheit (94) zum Anwenden einer Oberflächenreinigung des Stahlbasisdrahtes vor dem Schritt des Walzens zum Entfernen einer Oberflächenschicht wie einer Oxidationsschicht aus dem Stahlbasisdraht (15) umfasst; und im Gebrauch stromabwärts des Walzwerks eine Biegeeinheit (98) zum Anwenden mehrerer Biegewirkungen auf den Stahlbasisdraht, um dessen Zugeigenschaften zu verbessern.

8. Herstellungsanordnung nach Anspruch 7, ferner mit einer Oberflächenschicht-Brecheinheit (93) stromaufwärts der Oberflächenreinigungseinheit (94) zum Anwenden eines Schritts des Oberflächenschicht-Bruchs zum Brechen einer Oberflächenschicht des Drahtes (15).

9. Herstellungsanordnung nach Anspruch 7 oder 8, ferner mit einer Kugelstrahleneinheit stromabwärts der Biegeeinheit zum Anwenden eines Schritts des Kugelstrahlens nach dem Schritt des Anwendens der Biegewirkungen.

10. Herstellungsanordnung nach einem der Ansprüche 7 bis 9, wobei die Biegeeinheit (98) mehrere aufeinanderfolgende Walzenräder (57, 58, 59, 60, 61) umfasst, die in einer einzigen Rotationsebene angeordnet sind, wobei jedes Walzenrad mittels einer Welle (77, 78, 79, 80, 81) rotierbar ist, so dass sie in der Rotationsebene mehrerer Walzenräder rotierbar ist, wobei die Walzenräder so angeordnet sind, dass sie im Gebrauch zum Bereitstellen der Biegewirkung der Stahlbasisdraht über oder mit wenigstens einem Teil des Umfangs jedes Rads bewegt wird.

11. Herstellungsanordnung nach Anspruch 10, wobei sich die Wellen (77, 78, 79, 80, 81) der Walzenräder (57, 58, 59, 60, 61) von der Rotationsebene abwechselnd quer zur Rotationsebene von Positionen entlang einer ersten (70) bzw. einer zweiten Linie (72) erstrecken, wobei die erste (70) und die zweite Linie (72) parallel zueinander und zur Rotationsebene sind, wobei für jeweils zwei aufeinanderfolgende Walzenräder die Summe der Radien der Walzenräder größer als oder gleich einem Abstand zwischen der ersten und der zweiten Linie ist, um die Biegewirkung auf den Stahlbasisdraht beim Bewegen über oder mit dem Umfang der Walzenräder zu erzwingen.

12. Herstellungsanordnung nach Anspruch 11, wobei die Wellen (77, 79, 81), die sich von der ersten Linie (70) erstrecken, durch eine erste Aufhängungseinheit strukturell verbunden sind, und wobei sich die Wellen (78, 80) von der zweiten Linie (72) strukturell durch eine zweite Aufhängungseinheit verbunden sind, wobei wenigstens eine der ersten und zweiten Aufhängungseinheiten einstellbar mit einer Struktur der Vorrichtung verbunden ist, um eine Einstellung des Abstands zwischen der ersten (70) und der zweiten Linie (72) im Gebrauch zu ermöglichen.

13. Herstellungsanordnung nach Anspruch 12, wobei eine oder mehrere der Wellen (77, 78, 79, 80, 81) einstellbar mit der ersten oder zweiten Aufhängungseinheit verbunden sind, um eine Einstellung der Position der einen oder mehreren Wellen entlang der ersten Welle oder zweiten Linie zu ermöglichen.

14. Herstellungsanordnung nach einem der Ansprüche 10 bis 13, wobei die Walzenräder (57, 58, 59, 60, 61) lösbar an den Wellen (77, 78, 79, 80, 81) aufgehängt sind, um deren Austausch zum Anpassen im Gebrauch eines Durchmessers eines oder mehrerer Walzenräder (57, 58, 59, 60, 61) zu ermöglichen.

## Revendications

1. Procédé de fabrication d'acier de renforcement pour le renforcement de structures en béton pour fournir ledit acier de renforcement présentant un rapport de résistance à la traction à limite élastique Rₘ/Rₑ d'au moins 1,08, et présentant un allongement uniforme en pourcentage à une force maximale A_{gt} d'au moins 5,0, ledit acier de renforcement présentant une forme allongée de longueur et section transversale arbitraires, ledit procédé comprenant les étapes de :
fourniture (2) d'un câble de base en acier (15) ; et
laminage (6) du câble de base en acier (15) pour modifier une dimension transversale de celui-ci, et pour créer un profil de liaison sur une surface dudit câble (15), dans lequel ladite étape de laminage (6) est une étape de laminage à froid ;
**caractérisé en ce que**, avant l'étape de laminage, le procédé comprend de plus une étape de :
rupture de couche de surface (3) pour rompre une couche de surface, et
nettoyage de surface (4) dudit câble de base en acier (15) pour éliminer la couche de surface dudit câble de base en acier (15) ; et
dans lequel, après ladite étape de laminage, le procédé comprend de plus une étape (8) d'application de plusieurs actions de courbure au câble de base en acier (15) pour améliorer les propriétés de traction de celui-ci.

2. Procédé selon la revendication 1, comprenant de plus une étape de grenaillage (9) après ladite étape d'application des actions de courbure.

3. Procédé selon la revendication 1 ou 2, dans lequel lesdites actions de courbure sont appliquées en déplaçant le câble de base en acier (15) à travers plusieurs roues de cylindres consécutives (57, 58, 59, 60, 61), dans lequel pour chaque roue de cylindre destinée à fournir l'action de courbure le câble de base en acier (15) est déplacé à travers ou avec au moins une partie d'une circonférence de la roue.

4. Procédé selon la revendication 3, dans lequel chaque roue de cylindre (57, 58, 59, 60, 61) peut tourner dans un plan de rotation des plusieurs roues de cylindres, chaque roue de cylindre pouvant tourner au moyen d'un arbre, et dans lequel à partir du plan de rotation des roues de cylindres les arbres s'étendent de manière alternée transversalement par rapport au plan de rotation à partir de positons le long d'une première et d'une seconde ligne respectivement, la première et la seconde ligne étant parallèles l'une à l'autre et au plan de rotation, dans lequel pour à chaque fois deux roues de cylindres consécutives la somme des rayons des roues de cylindres est supérieure ou égale à une distance entre les première et seconde lignes pour forcer ladite action de courbure sur le câble de base en acier lors du déplacement du câble à travers ou avec la circonférence des roues de cylindres.

5. Procédé selon l'une quelconque des revendications précédentes, dans lequel l'étape (8) d'application de plusieurs actions de courbure comprend l'application d'au moins trois actions de courbure.

6. Procédé selon l'une quelconque des revendications précédentes, dans lequel ladite étape supplémentaire de nettoyage de surface comprend au moins une étape choisie dans un groupe comprenant le brossage, le polissage, le bobinage du câble de base en acier, un traitement chimique, tel qu'une coloration, ou un jet de fluide haute pression pour nettoyer le câble de base en acier.

7. Dispositif de fabrication pour la fabrication d'acier de renforcement pour le renforcement de structures en béton présentant un rapport de résistance à la traction à limite élastique Rₘ/Rₑ d'au moins 1,08, et présentant un allongement uniforme en pourcentage à une force maximale A_{gt} d'au moins 5,0, en utilisant un procédé selon au moins une des revendications 1-6, ledit dispositif comprenant :
une unité d'amenée pour recevoir un câble de base en acier (15) ; et
une unité de laminoir (96) pour appliquer une étape de laminage à froid pour laminer le câble de base en acier pour modifier une dimension transversale de celui-ci, et pour créer un profil de liaison sur une surface dudit câble ;
ledit dispositif **caractérisé en ce qu'**il comprend de plus, dans une utilisation en amont dudit laminoir (96), une unité de nettoyage de surface (94) pour appliquer un nettoyage de surface dudit câble de base en acier avant ladite étape de laminage pour éliminer une couche de surface telle qu'une couche d'oxydation dudit câble de base en acier (15) ; et, dans une utilisation en aval dudit laminoir, une unité de courbure (98) pour appliquer plusieurs actions de courbure au câble de base en acier pour améliorer les propriétés de traction de celui-ci.

8. Dispositif de fabrication selon la revendication 7, comprenant de plus une unité de rupture de couche de surface (93) en amont de ladite unité de nettoyage de surface (94) pour appliquer une étape de rupture de couche de surface pour rompre une couche de surface du câble (15).

9. Dispositif de fabrication selon la revendication 7 ou 8, comprenant de plus une unité de grenaillage en aval de ladite unité de courbure pour appliquer une étape de grenaillage après ladite étape d'application des actions de courbure.

10. Dispositif de fabrication selon l'une quelconque des revendications 7-9, l'unité de courbure (98) comprenant plusieurs roues de cylindres consécutives (57, 58, 59, 60, 61) disposées dans un seul plan de rotation, dans lequel chaque roue de cylindre peut tourner au moyen d'un arbre (77, 78, 79, 80, 81) afin de pouvoir tourner dans le plan de rotation des plusieurs roues de cylindres, lesdites roues de cylindres étant placées de sorte que dans une utilisation pour fournir l'action de courbure le câble de base en acier est déplacé à travers ou avec au moins une partie de la circonférence de chaque roue.

11. Dispositif de fabrication selon la revendication 10, dans lequel à partir du plan de rotation les arbres (77, 78, 79, 80, 81) des roues de cylindres (57, 58, 59, 60, 61) s'étendent de manière alternée transversalement par rapport au plan de rotation à partir de positions le long d'une première (70) et d'une seconde ligne (72) respectivement, la première (70) et la seconde ligne (72) étant parallèles l'une à l'autre et au plan de rotation, dans lequel pour à chaque fois deux roues de cylindres consécutives la somme des rayons des roues de cylindres est supérieure ou égale à une distance entre les première et secondes lignes pour forcer ladite action de courbure sur le câble de base en acier lors du déplacement du câble à travers ou avec la circonférence des roues de cylindres.

12. Dispositif de fabrication selon la revendication 11, dans lequel les arbres (77, 79, 81) s'étendant à partir de la première ligne (70) sont structurellement connectés par une première unité de suspension, et dans lequel les arbres (78, 80) s'étendant à partir de la seconde ligne (72) sont structurellement connectés par une seconde unité de suspension, dans lequel au moins une des première et seconde unités de suspension est connectée de manière ajustable à une structure de l'appareil afin de permettre un ajustement de la distance entre les première (70) et seconde lignes (72) lors de l'utilisation.

13. Dispositif de fabrication selon la revendication 12, dans lequel un ou plusieurs des arbres (77, 78, 79, 80, 81) est connecté de manière ajustable à la première ou seconde unité de suspension, pour permettre un ajustement de la position des uns ou plusieurs arbres le long de la première ou seconde ligne respectivement.

14. Dispositif de fabrication selon l'une quelconque des revendications 10-13, dans lequel les roues de cylindres (57, 58, 59, 60, 61) sont suspendues aux arbres (77, 78, 79, 80, 81) de manière détachable de sorte à permettre un remplacement de celles-ci, pour adapter un diamètre d'une ou plusieurs roues de cylindres (57, 58, 59, 60, 61) lors de l'utilisation.
